# EUROPEAN PATENT SPECIFICATION

(11) **EP 0 456 659 B1**
(45) Date of publication and mention of the grant of the patent: **30.06.2004**
(21) Application number: 90902057.0
(22) Date of filing: 16.01.1990
(51) Int. Cl.: G03G 9/135, G03G 9/13, G03G 9/12

(54) **CHARGE DIRECTOR COMPOSITION**
LADUNGSSTEUERUNGSZUSAMMENSETZUNG
COMPOSITION DE CONTROLE DE CHARGE

(30) Priority: 06.02.1989 US 306155
(43) Date of publication of application: 21.11.1991
(73) Proprietor: Hewlett-Packard Indigo B.V., 6221 SH Maastricht (NL)
(72) Inventor: LANDA, Benzion, Edmonton, Alberta T5J0J0 (CA); ALMOG, Yaacov, 76 100 Rehovot (IL)
(74) Representative: Leadbetter, Benedict
(86) International application number: PCT/US1990/000155
(87) International publication number: WO 1990/008983

(56) References cited:
- EP-A- 0 001 103
- EP-A- 0 242 806
- DE-A- 1 930 783
- DE-U- 9 193 078
- FR-A- 2 015 892

## Description

### BACKGROUND OF THE INVENTION

The present invention relates to liquid developer electrostatic photocopying and more particularly to a method of stabilizing charge director solutions and a new stabilized charge director composition.

Processes for forming electrostatic images, existing as electrostatic charge patterns upon a substrate, are well known. In electrostatic printing or copying, a photoconductive imaging surface is first provided with a uniform electrostatic charge, typically by moving the imaging surface past a charge corona at a uniform velocity. The imaging surface is then exposed to an optical image of an original to be copied. This optical image selectively discharges the imaging surface in a pattern to form a latent electrostatic image. In the case of an original bearing dark print on a light background, this latent image consists of substantially undischarged "print" portions corresponding to the graphic matter on the original, amidst a "background" portion that has been substantially discharged by exposure to light. The latent image is developed by exposure to oppositely charged, pigmented, toner particles, which deposit on the print portions of the latent image in a pattern corresponding to that of the original.

In liquid developer photocopiers, these charged toner particles are suspended in a liquid developer comprising a carrier liquid, toner particles and charge directors. The entire latent electrostatic image is covered with a thin film of liquid developer from a liquid developer reservoir. The charged toner particles in the liquid developer migrate to the oppositely charged "print" portions of the latent image to form a pattern on the photoconductive surface. This pattern, and the corresponding toner particles, are then transferred to a sheet to produce a visible image. Any liquid developer remaining on the photoconductive surface after this process is recycled back into the liquid developer reservoir.

EP-A-001103 describes a method of producing a charge director from a number of components, including a monomer species which is polarised during the process. The charge director is a copolymer soluble in a carrier liquid, and is composed of 1-50% by weight of N-vinyl-2-pyrrolidine and 50 - 99% by weight methacrylic acid ester.

DE-A-1930783 describes a polymeric material, an alkylated polymer of heterocyclic vinyl monomer, capable of imparting negative working characteristics to an electrostatic toner.

Charge director plays an important role in the developing process described above. The charge director is a chemical species, either molecular or ionic, which acts to control the polarity and charge on the toner particles. The charge director creates charged species causing charging of the imaging material to ensure that the toner particles will be deposited and migrate in such a way as to form the desired image on the imaging surface. Counter ions are also created to keep the liquid developer substantially electrically neutral overall. The present invention may be practised with any number of charge directors, of which lecithin and barium petronate are examples.

One of the major problems concerning the material used as charge directors is the degradation of the charge carrying species under the application of the electric field created during the electrophoretic development process. Degradation of the charge carrying species also occurs during replenishment of developer with carrier liquid due to dilution of the charge director. Degradation of the charge carrying species destabilizes the liquid developer electrically. Since stable electrical characteristics of the liquid developer are important to achieve a high quality image, particularly when a large number of impressions are to be produced without changing the liquid developer dispersion, degradation of the charge carrying species results in poor copy quality.

It is believed that in many liquid developers the charge director molecules form inverse micelles. An example of these micelles is shown in Figure 1. The micelles are formed by aggregation such that the polar portions of the charge director molecules point inside, and the nonpolar portions point outside to decrease the overall surface energy of the system. These micelles may solubilize ions generated by the disassociation of the charge director molecules. It is believed that the solubilization of ions by the charge director micelles is due to the formation within and around the micelles, of a microenvironment having a higher dielectric constant. The solubilization of ions by the charge director micelles results in micelles containing a charged species in their center. Some of the micelles have a positive species in the center and others have a negative species in the center. We believe that during the electrophoretic developing process these micelles rupture under the influence of the electric field created by the charged photoconductive surface. The exact mechanism of the rupturing is not known. The rupture of the micelles changes the electrical properties of the liquid developer solution by freeing the charged species in the center of the micelles which, due to their relatively strong positive and negative charges and the low dielectric constant of the carrier liquid, tend to reassociate with each other to form electrically neutral compounds. The formation of these electrically neutral compounds changes the overall electrical properties of the liquid developer. The change in electrical properties of the liquid developer changes the toner particle dispersion in the liquid developer and the number of the charge-carrying species resulting in a degradation in copy quality.

We also believe that the micelles rupture when the liquid developer dispersion in a photocopier is replenished by the addition of new carrier liquid. Again, the exact mechanism is not known. The effect of this rupturing is manifested in an instability of the charge-carrying species in the system. Again, the overall result is a degradation in copy quality.

Accordingly, one object of the present invention is a charge director composition which will resist degradation under the influence of an electric field.

Another object of the present invention is a charge director composition which will resist degradation during the replenishment of carrier liquid in a liquid developer dispersion.

A further object of the present invention is a charge director solution which will resist destabilization.

### BRIEF DESCRIPTION OF THE DRAWINGS

Figure 1 is an idealized depiction of charge director micelles.
Figure 2 is a graphic representation of the current in a lecithin solution for 4 successive electric pulses.
Figure 3 is a graphic representation of the conductivity kinetics under dilution of lecithin and the material of the present invention.
Figure 4 is a graphic representation of the stability of various charge director compositions of the present invention.
Figure 5 shows the absolute change in conductivity during a long developing run for a 21% coverage target for lecithin and a charge director of the present invention.

### SUMMARY OF THE INVENTION

The present invention is directed to a method of stabilizing a charge director solution as claimed in claim 1 wherein a charge director, a carrier liquid, and a polar monomer molecules are mixed, and subsequently the monomer molecules are polymerized. An initiator species is used to begin the polymerization and the reaction is allowed to proceed to substantial completion. We believe that the result is a chemical incorporation of a polar polymer, species into the core of the charge director micelles. The polar species stabilizes the core of the micelles and reduces the possibility of the micelle rupturing.

In accordance with the present invention, charge director micelles are associated with insoluble polymer molecules so that the charged species are more stable and less susceptible to degradation. It will be appreciated that by reducing the degradation of the charged species of the liquid developer composition the images formed by the developer will be denser over a longer period of usage, since the presence of the charged species is essential to the electrophoretic imaging process.

The present invention is also directed to a charge director composition as claimed in claim 11 and to a liquid developer as claimed in claim 19.

### Detailed Description

In our invention, a charge director, a solvent, and polar monomer molecules are mixed, and subsequently the monomer molecules are polymerized. An initiator is used to begin the polymerization and the reaction is allowed to proceed to substantial completion. While the polymer which is formed is not soluble, the monomeric molecules of the present invention are soluble in the solvent containing the charge director. The charge director, which is at least partially present as micelles, acts as a surfactant for the polymerization of the monomer species. It is believed the monomer species clings to the micelle and polymerizes in the core of the micelle.

The selected solvent may be any suitable solvent in which the necessary polymerization may occur. Many nonpolar solvents will work well in the present invention, including: Isopar (a trademarked product of the Exxon Corporation), Isoparafine, hexane, cyclohexane, t-butylbenzene, 2,2,4-trimethylpentane, and normal paraffins. The monomer species chosen may be any unsaturated monomer that is soluble in the selected solvent and polymerizes in the solvent in the presence of an appropriate initiator. It is believed a large number of unsaturated molecules will work well in the present invention as a monomer, but certain species should work especially well, including 1-vinyl-2-pyrrolidone, 2-vinyl pyridine, vinylfuran, and methylmethacrylate.

It is believed that the initiator may be any one of a large number of species which will initiate a polymerization reaction, including azobisbutyronitrile, benzoyl peroxide, triphenylazobenzene, cumene hydroperoxide, and t-butyl peracetate.

In one preferred embodiment of the present invention, Isopar is heated to approximately 50 degrees C in a reaction vessel fitted with a reflux condenser The reaction is run under a nitrogen atmosphere. Lecithin is slowly mixed into the Isopar. The solution is heated to about 80-90 degrees C and 1-vinyl-2-pyrrolidone is added, followed by a polymerization initiator, e.g., azobisbutyronitrile. The temperature is kept constant, and the reaction is allowed to proceed for about 24 hours. The charge director composition formed by this process will be less subject to degradation of the charge-carrying species than a composition lacking the stabilizing polymer molecules. This superior resistance to degradation will be exhibited both when an electric current is applied to the composition, and when the composition is diluted with solvent (Isopar).

It is preferred to use a nonpolar solvent in which the 1-vinyl-2-pyrrolidone monomer is soluble, but the polymer is insoluble. The solvent should boil at a significantly higher temperature than 90°C, so that it will remain liquid under the reaction conditions. It is believed that, as the polymerization reaction progresses, the polymer molecules will reach a critical length above which they are insoluble in the solvent; a very fine dispersion of these polymer molecules in the solvent results, and the charge director micelles form around the polymer molecules. The micelles in turn are rigidized and stabilized by the polymer molecules. The critical percent of vinyl pyrrolidone polymer needed to obtain a large stabilization effect is between about 5-9% on a weight-to-weight basis with respect to the charge director solids. With a polymer concentration of 9% or more, very little degradation of the charged species occurs upon dilution with solvent or the imposition of an electric field. Below a 5% polymer concentration, however, a significant amount of degradation will occur. The present invention is further illustrated by, but not limited to, the following examples.

### EXAMPLE I

Under a nitrogen atmosphere, 1400 grams of Isopar-H was heated to 50 deg. C in a 4-necked, 2 liter, mechanically stirred glass reactor fitted with a reflux condenser. 600 grams of lecithin was dissolved in the Isopar-H by slow addition and stirring. The Isopar-H/Lecithin solution was then heated to 80°C and then 102 grams of 1-vinyl-2-pyrrolidone was added to the solution. Three grams of azobisbutyronitrile suspended in 10-20 ml. of Isopar-H was then added, and the reaction allowed to proceed for 24 hours to completion.

### EXAMPLE II

500 grams Isopar-H, 10 grams of lecithin, and 1.7 grams 1-vinyl-2-pyrrolidone were mixed at 90 deg. C in a 4-necked glass roundbottom flask under an N₂ atmosphere. 0.5 grams azobisbutyronitrile was dispersed in 20 grams of Isopar and added. The reaction was allowed to proceed for 17-1/2 hours. The resulting solution was clear, and somewhat darker than a solution of lecithin in Isopar.

The advantages of the present invention are illustrated by the following experimental results.

Table 1 and Figure 2 show the results of our experiment on the effect of an applied electric field to a common unstabilized charge director, lecithin, solution. In the experiment 800 V. DC pulses were sequentially applied to a cell containing a lecithin solution for 4 seconds and the charge transport of the lecithin solution for each pulse was measured. Table 1 shows the charge transport in the solution for each pulse. Figure 2 is a graphic representation of the current in the Lantern solution during the time period of the pulse. As shown in Table 1 and Figure 2 the application of an electric pulse to a charge director solution changes the electrical properties of the solution. The applied electric pulse of the experiment is similar to the electric field created during the copying process. Thus, the effect of the electric pulse on the lecithin solution resembles the effect of the electric field created during the copying process of the liquid developer solution.

Figure 3 show the conductivity of a composition comprising 17% monomer stabilized species by weight with respect to charge director solids, according to the present invention as compared to a lecithin control, in both cases after addition of a carrier liquid such as Isopar H. As shown in Figure 3, the conductivity of the stabilized composition in Isopar remains relatively constant with time, while that of the control decreases with time. Thus, the stabilized composition of the present invention is advantageous for use in a photocopier since the conductivity will not change appreciably with time.

Figure 4 shows the results of a similar experiment on various stabilized charge director compositions according to the present invention. In this experiment 4, 800 V. DC pulses were sequentially applied to a cell containing a charge director solution and the total charge transport in the cell was measured for each pulse. The control charge director solution was an unstabilized lecithin solution as used in the above-mentioned experiment. Five stabilized charge director solutions made according to the present invention were also tested. Each charge director solution was made with a different percentage of the monomer stabilizing species. As shown in Figure 4, the charge director solution should comprise between 5% and 9% by weight with respect to charge director solids or more of the monomer stabilizing species to achieve a high degree of charge transport constancy. As also shown in Figure 4, little degradation in charge transport is maintained by a charge director composition comprising 17% monomer stabilizing species by weight with respect to charge director solids.

Figure 5 shows the results of an experiment on the decrease in conductivity of a charge director solution during continuous electrophotocopier operation with no paper feed. The lecithin charge director solution shown on the chart is an unstabilized ordinary charge director solution. The other charge director is made according to example 1 of the present invention comprising 17% monomer stabilizing species by weight with respect to charge director solids. As discussed in a preceding section, we believe that during the electrophotographic process unstabilized charge director micelles rupture, causing the decrease in the number of charge species, and thus a decrease in bulk conductivity of the liquid developer and a degradation in copy quality. As shown in Figure 5, the unstabilized lecithin solution had a decrease of an 18picomho/cm in conductivity during the electrophotocopier operation. The solution comprising 17% monomer stabilizing species by weight with respect to charge director solids, made according to example 1 of the present invention, however, showed only a 4picomho/cm decrease in conductivity during continuous electrophotocopier operation.

It should be understood that the foregoing descriptions are for the purpose of illustration only and that the invention includes all modifications falling within the scope of the appended claims.

## Claims

1. A method for stabilizing a charge director solution for an electrophotographic liquid developer comprising the steps of:
mixing a charge director with polar monomer molecules in a carrier liquid in which they are both soluble,
initiating a polymerization reaction among said monomer molecules; and
allowing said polymerization reaction to progress to completion to thereby associate the polymer thus formed with said charge director.

2. A method as claimed in claim 1, wherein the polar monomer species is 1-vinyl-2-pyrrolidine.

3. A method as claimed in claim 1 or 2, wherein the charge director is lecithin.

4. A method as claimed in claim I, 2 or 3, wherein the solvent is a non-polar organic compound comprising a mixture of compounds.

5. A method as claimed in claim 4, wherein said non-polar organic solvent is Isopar-H.

6. A method as claimed in any preceding claim, wherein the reaction is initiated by the addition of azobisbutyronitrile.

7. A method as claimed in any preceding claim, wherein the reaction is run under an atmosphere of nitrogen, argon, or another inert gas.

8. A method as claimed in any preceding claim, wherein the polar monomer species comprises at least 5% by weight with respect to charge director solids.

9. A method as claimed in claim 8, wherein the polar monomer species comprises 5% to 9% by weight with respect to charge director solids.

10. A method as claimed in claim 8, wherein the polar monomer species comprises between 10% and 17% by weight with respect to the charge director solids.

11. A charge director composition for an electrophotographic liquid developer comprising a carrier liquid, a polar polymer insoluble in said carrier liquid, and a charge director soluble in said carrier liquid, said charge direction being stabilized by association with the polymer, and obtainable by the process comprising the steps of:
mixing a charge director with a solvent and a polar monomer molecules;
initiating a polymerization reaction among said monomer molecules; and
allowing said polymerization reaction to progress to completion to thereby associate the polymer thus formed with said charge director.

12. A charge director composition as claimed in claim 11, wherein said solvent is a non-polar organic compound or mixture of compounds.

13. A charge director composition as claimed in claim 12, wherein the solvent is Isopar-H.

14. A charge director composition as claimed in any one of claims 11 to 13, wherein the charge director is lecithin.

15. A charge director composition as claimed in any one of claims 11 to 14, wherein the polymer is polyvinylpyrrolidone.

16. A charge director composition as claimed in claim 11 or any claim dependent thereon, wherein the polar monomer species comprises at least 5% by weight with respect to charge director solids.

17. A charge director composition as claimed in claim 16, wherein the polar monomer species comprises 5% to 9% by weight with respect to charge director solids.

18. A charge director composition as claim in claim 16, wherein the polar monomer species comprises between 10% and 17% by weight with respect to charge director solids.

19. A electropholographic liquid developer comprising a carrier liquid, toner particles and a charge director soluble in the carrier liquid, **characterised in that** the charge director is stabilized by association with a polar polymer that is insoluble in the carrier liquid, said liquid developer being obtainable by the process comprising the steps of:
mixing a charge director with a solvent and a polar monomer molecules;
initiating a polymerization reaction among said monomer molecules; and
allowing said polymerization reaction to progress to completion to thereby associate the polymer thus formed with said charge director.

20. The liquid developer of claim 19, wherein the charge director is lecithin.

21. The liquid developer of claim 19 or 20, wherein the polymer is polyvinylpyrrolidone.

22. The liquid developer of claim 19, wherein the charge director is at least partially present in the form of micelles and acts as a surfactant for the polymerization of the monomer species.

23. The liquid developer of claim 19 or 22, wherein the solvent is the carrier liquid.

## Patentansprüche

1. Ein Verfahren zum Stabilisieren einer Ladungsdirektorlösung für einen elektrophotographischen Flüssigentwickler, mit folgenden Schritten:
Mischen eines Ladungsdirektors mit Polar-Monomer-Molekülen in einer Trägerflüssigkeit, in der beide löslich sind;
Einleiten einer Polymerisierungsreaktion unter den Monomer-Molekülen; und
Ermöglichen, daß die Polymerisierungsreaktion bis zum Abschluß fortfahren kann, um dadurch das so erzeugte Polymer dem Ladungsdirektor zuzuordnen.

2. Ein Verfahren gemäß Anspruch 1, bei dem die polare Monomer-Spezies 1-Vinyl-2-Pyrrolidin ist.

3. Ein Verfahren gemäß Anspruch 1 oder 2, bei dem der Ladungsdirektor Lecithin ist.

4. Ein Verfahren gemäß einem der Ansprüche 1, 2 oder 3, bei dem das Lösungsmittel eine nicht-polare organische Verbindung ist, die eine Mischung von Verbindungen aufweist.

5. Ein Verfahren gemäß Anspruch 4, bei dem das nicht-polare organische Lösungsmittel Isopar-H ist.

6. Ein Verfahren gemäß einem der vorhergehenden Ansprüche, bei dem die Reaktion durch die Zugabe von Azobisbutyronitril eingeleitet wird.

7. Ein Verfahren gemäß einem der vorhergehenden Ansprüche, bei dem die Reaktion unter einer Atmosphäre aus Stickstoff, Argon oder einem weiteren Edelgas abläuft.

8. Ein Verfahren gemäß einem der vorhergehenden Ansprüche, bei dem die polare Monomer-Spezies zumindest fünf Gewichtsprozent in bezug auf Ladungsdirektor-Feststoffe aufweist.

9. Ein Verfahren gemäß Anspruch 8, bei dem die polare Monomer-Spezies 5 bis 9 Gewichtsprozent in bezug auf Ladungsdirektor-Feststoffe aufweist.

10. Ein Verfahren gemäß Anspruch 8, bei dem die polare Monomer-Spezies zwischen 10 und 17 Gewichtsprozent in bezug auf die Ladungsdirektor-Feststoffe aufweist.

11. Eine Ladungsdirektor-Zusammensetzung für einen elektrophotographischen Flüssigentwickler, die eine Trägerflüssigkeit, ein Polar-Polymer, das in der Trägerflüssigkeit unlöslich ist, und einen Ladungsdirektor aufweist, der in der Trägerflüssigkeit löslich ist, wobei der Ladungsdirektor durch eine Zuordnung zu dem Polymer stabilisiert ist und durch den Vorgang erhältlich ist, der folgende Schritte aufweist:
Mischen eines Ladungsdirektors mit einem Lösungsmittel und Polar-Monomer-Molekülen;
Einleiten einer Polymerisierungsreaktion unter den Monomer-Molekülen; und
Ermöglichen, daß die Polymerisierungsreaktion bis zum Abschluß fortfahren kann, um dadurch das so erzeugte Polymer dem Ladungsdirektor zuzuordnen.

12. Eine Ladungsdirektor-Zusammensetzung gemäß Anspruch 11, bei der das Lösungsmittel eine nicht-polare organische Verbindung oder Mischung von Verbindungen ist.

13. Eine Ladungsdirektor-Zusammensetzung gemäß Anspruch 12, bei der das Lösungsmittel Isopar-H ist.

14. Eine Ladungsdirektor-Zusammensetzung gemäß einem der Ansprüche 11 bis 13, bei der der Ladungsdirektor Lecithin ist.

15. Eine Ladungsdirektor-Zusammensetzung gemäß einem der Ansprüche 11 bis 14, bei der das Polymer Polyvinylpyrrolidon ist.

16. Eine Ladungsdirektor-Zusammensetzung gemäß Anspruch 11 oder einem davon abhängigen Anspruch, bei der die polare Monomer-Spezies zumindest fünf Gewichtsprozent in bezug auf Ladungsdirektor-Feststoffe aufweist.

17. Eine Ladungsdirektor-Zusammensetzung gemäß Anspruch 16, bei der die polare Monomer-Spezies 5 bis 9 Gewichtsprozent in bezug auf Ladungsdirektor-Feststoffe aufweist.

18. Eine Ladungsdirektor-Zusammensetzung gemäß Anspruch 16, bei der die polare Monomer-Spezies zwischen 10 und 17 Gewichtsprozent in bezug auf die Ladungsdirektor-Feststoffe aufweist.

19. Ein elektrophotographischer Flüssigentwickler, der eine Trägerflüssigkeit, Tonerteilchen und einen Ladungsdirektor aufweist, der in der Trägerflüssigkeit löslich ist, **dadurch gekennzeichnet, daß** der Ladungsdirektor durch eine Zuordnung zu einem Polar-Polymer stabilisiert ist, das in der Trägerflüssigkeit unlöslich ist, wobei der Flüssigentwickler durch den Vorgang erhältlich ist, der folgende Schritte aufweist:
Mischen eines Ladungsdirektors mit einem Lösungsmittel und Polar-Monomer-Molekülen;
Einleiten einer Polymerisierungsreaktion unter den Monomer-Molekülen; und
Ermöglichen, daß die Polymerisierungsreaktion bis zum Abschluß fortfahren kann, um dadurch das so erzeugte Polymer dem Ladungsdirektor zuzuordnen.

20. Der Flüssigentwickler gemäß Anspruch 19, bei dem der Ladungsdirektor Lecithin ist.

21. Der Flüssigentwickler gemäß Anspruch 19 oder 20, bei dem Polymer Polyvinylpyrrolidon ist.

22. Der Flüssigentwickler gemäß Anspruch 19, bei dem der Ladungsdirektor zumindest teilweise in der Form von Mizellen vorliegt und als ein oberflächenaktives Mittel für die Polymerisierung der Monomer-Spezies wirkt.

23. Der Flüssigentwickler gemäß Anspruch 19 oder 22, bei dem das Lösungsmittel die Trägerflüssigkeit ist.

## Revendications

1. Procédé de stabilisation d'une solution de contrôle de charge pour un révélateur électrophotographique liquide comprenant les étapes consistant à :
mélanger un contrôle de charge avec des molécules de monomère polaire dans un liquide de transport dans lequel ils sont tous deux solubles ;
initier une réaction de polymérisation parmi lesdites molécules de monomère ; et
laisser progresser ladite réaction de polymérisation jusqu'à son terme pour associer ainsi le polymère ainsi formé avec ledit contrôle de charge.

2. Procédé selon la revendication 1, dans lequel l'espèce de monomère polaire est de la 1-vinyle-2-pyrrolidine.

3. Procédé selon la revendication 1 ou 2, dans lequel le contrôle de charge est de la lécithine.

4. Procédé selon la revendication 1, 2 ou 3, dans lequel le solvant est un composé organique non polaire comprenant un mélange de composés.

5. Procédé selon la revendication 4, dans lequel ledit solvant organique non polaire est de l'Isopar-H.

6. Procédé selon l'une quelconque des revendications précédentes, dans lequel la réaction est initiée par l'ajout d'azobisbutyronitrile.

7. Procédé selon l'une quelconque des revendications précédentes, dans lequel la réaction est conduite dans une atmosphère d'azote, d'argon ou d'un autre gaz inerte.

8. Procédé selon l'une quelconque des revendications précédentes, dans lequel l'espèce monomère polaire comprend au moins 5 % en poids par rapport aux matières solides de contrôle de charge.

9. Procédé selon la revendication 8, dans lequel l'espèce monomère polaire comprend de 5 % à 9 % en poids par rapport aux matières solides de contrôle de charge.

10. Procédé selon la revendication 8, dans lequel l'espèce monomère polaire comprend de 10 % à 17 % en poids par rapport aux matières solides de contrôle de charge.

11. Composition de contrôle de charge pour un révélateur électrophotographique liquide comprenant un liquide de transport, un polymère polaire insoluble dans ledit liquide de transport, et un contrôle de charge soluble dans ledit liquide de transport, ledit contrôle de charge étant stabilisé par association avec le polymère, et susceptible d'être obtenu par le procédé comprenant les étapes consistant à :
mélanger un contrôle de charge avec un solvant et des molécules de monomère polaire ;
initier une réaction de polymérisation parmi lesdites molécules de monomère ; et
laisser progresser ladite réaction de polymérisation jusqu'à son terme pour associer ainsi le polymère ainsi formé avec ledit contrôle de charge.

12. Composition de contrôle de charge selon la revendication 11, dans laquelle ledit solvant est un composé organique non polaire ou un mélange de composés.

13. Composition de contrôle de charge selon la revendication 12, dans laquelle le solvant est de l'Isopar-H.

14. Composition de contrôle de charge selon l'une quelconque des revendications 11 à 13, dans laquelle le contrôle de charge est de la lécithine.

15. Composition de contrôle de charge selon l'une quelconque des revendications 11 à 14, dans laquelle le polymère est du polyvinylpyrrolidone.

16. Composition de contrôle de charge selon la revendication 11 ou toute revendication dépendante de celle-ci, dans laquelle l'espèce monomère polaire comprend au moins 5 % en poids par rapport aux matières solides de contrôle de charge.

17. Composition de contrôle de charge selon la revendication 16, dans laquelle l'espèce monomère polaire comprend de 5 % à 9 % en poids par rapport aux matières solides de contrôle de charge.

18. Composition de contrôle de charge selon la revendication 16, dans laquelle l'espèce monomère polaire comprend de 10 % à 17 % en poids par rapport aux matières solides de contrôle de charge.

19. Révélateur électrophotographique liquide comprenant un liquide de transport, des particules de toner et un contrôle de charge soluble dans le liquide de transport, **caractérisé en ce que** le contrôle de charge est stabilisé par association avec un polymère polaire qui est insoluble dans le liquide de transport, ledit révélateur liquide susceptible d'être obtenu par le procédé comprenant les étapes consistant à :
mélanger un contrôle de charge avec un solvant et des molécules de monomère polaire ;
initier une réaction de polymérisation parmi lesdites molécules de monomère ; et
laisser progresser ladite réaction de polymérisation jusqu'à son terme pour associer ainsi le polymère ainsi formé avec ledit contrôle de charge.

20. Révélateur liquide selon la revendication 19, dans lequel le contrôle de charge est de la lécithine.

21. Révélateur liquide selon la revendication 19 ou 20, dans lequel le polymère est du polyvinylpyrrolidone.

22. Révélateur liquide selon la revendication 19, dans lequel le contrôle de charge est au moins partiellement présent sous la forme de micelles et agit comme un agent de surface pour la polymérisation de l'espèce monomère.

23. Révélateur liquide selon la revendication 19 ou 22, dans lequel le solvant est le liquide de transport.
